



US012104327B2

(12) **United States Patent**  
**Langford et al.**

(10) **Patent No.:** **US 12,104,327 B2**  
(45) **Date of Patent:** **Oct. 1, 2024**

(54) **TISSUES AND PAPER TOWELS  
INCORPORATING SURFACE ENHANCED  
PULP FIBERS AND METHODS OF MAKING  
THE SAME**

(71) Applicant: **Domtar Paper Company, LLC**, Fort Mill, SC (US)

(72) Inventors: **Bradley Langford**, Fort Mill, SC (US); **David Lloyd**, Fort Mill, SC (US); **Brian Ranson**, Fort Mill, SC (US); **Gwen Johnston**, Fort Mill, SC (US); **Dale Kavalew**, Fort Mill, SC (US)

(73) Assignee: **Domtar Paper Company, LLC**, Fort Mill, SC (US)

(\*) Notice: Subject to any disclaimer, the term of this patent is extended or adjusted under 35 U.S.C. 154(b) by 148 days.

(21) Appl. No.: **17/754,087**

(22) PCT Filed: **Sep. 23, 2020**

(86) PCT No.: **PCT/US2020/052146**

§ 371 (c)(1),  
(2) Date: **Mar. 23, 2022**

(87) PCT Pub. No.: **WO2021/061723**

PCT Pub. Date: **Apr. 1, 2021**

(65) **Prior Publication Data**

US 2022/0333312 A1 Oct. 20, 2022

**Related U.S. Application Data**

(60) Provisional application No. 62/904,397, filed on Sep. 23, 2019.

(51) **Int. Cl.**  
**D21H 27/00** (2006.01)  
**D21D 1/20** (2006.01)

(Continued)

(52) **U.S. Cl.**  
CPC ..... **D21H 27/007** (2013.01); **D21D 1/20** (2013.01); **D21F 11/14** (2013.01); **D21H 27/38** (2013.01)

(58) **Field of Classification Search**

CPC .... D21H 27/007; D21H 27/38; D21H 27/005; D21D 1/20; D21C 9/007; D21F 11/14  
See application file for complete search history.

(56) **References Cited**

**U.S. PATENT DOCUMENTS**

3,098,785 A 7/1963 Meiler  
3,388,037 A 6/1968 Asplund et al.  
(Continued)

**FOREIGN PATENT DOCUMENTS**

AU 2015218812 B2 4/2017  
AU 2013305802 B2 5/2017  
(Continued)

**OTHER PUBLICATIONS**

Korean Notice of Preliminary Rejection in related Korean Patent Application No. KR10-2023-7022380 dated Aug. 21, 2023 with English Translation.

(Continued)

*Primary Examiner* — Jose A Fortuna

(74) *Attorney, Agent, or Firm* — Troutman Pepper Hamilton Sanders LLP; Alison L. McCarthy; Celeste K. Walker

(57) **ABSTRACT**

Paper products can comprise a first plurality of fibers that are hardwood fibers and a second plurality of fibers that include softwood fibers and surface enhanced pulp fibers (SEPF). The paper product can include one or more first fiber layers that comprise the first fibers, at least one of the first fiber layer(s) defining one of opposing upper and lower surfaces of the paper product, and one or more second fiber layers that comprise the second fibers. When a tissue, by weight,

(Continued)



between 50% and 80% of the tissue's fibers can be the first fibers and at least 20% of the tissue's fibers can be the second fibers. The tissue's basis weight can be less than or equal to 21 gsm per ply.

## 15 Claims, 5 Drawing Sheets

(51) Int. Cl.  
*D21F 11/14* (2006.01)  
*D21H 27/38* (2006.01)

(56) **References Cited**

U.S. PATENT DOCUMENTS

|             |      |         |                                       |
|-------------|------|---------|---------------------------------------|
| 3,519,211   | A    | 7/1970  | Marsan et al.                         |
| 3,708,130   | A    | 1/1973  | Perry                                 |
| 3,794,558   | A    | 2/1974  | Back                                  |
| 3,873,412   | A    | 3/1975  | Charters et al.                       |
| 3,891,499   | A    | 6/1975  | Kato et al.                           |
| 3,920,508   | A    | 11/1975 | Yonemori                              |
| 3,966,543   | A    | 6/1976  | Cayle et al.                          |
| 4,012,279   | A    | 3/1977  | Selander et al.                       |
| 4,054,625   | A    | 10/1977 | Kozlowski et al.                      |
| 4,247,362   | A    | 1/1981  | Williams                              |
| 4,337,116   | A    | 6/1982  | Foster et al.                         |
| 4,635,864   | A    | 1/1987  | Peterson et al.                       |
| 4,895,019   | A    | 1/1990  | Lehmikangas et al.                    |
| 1,925,530   | A    | 5/1990  | Sinclair et al.                       |
| 5,110,412   | A    | 5/1992  | Fuentes et al.                        |
| 5,248,099   | A    | 9/1993  | Lahner et al.                         |
| 5,308,449   | A    | 5/1994  | Fuentes et al.                        |
| 5,695,136   | A    | 12/1997 | Rohden et al.                         |
| 5,731,080   | A    | 3/1998  | Cousin et al.                         |
| 5,824,364   | A    | 10/1998 | Cousin et al.                         |
| 5,954,283   | A *  | 9/1999  | Matthew ..... B02C 7/12<br>241/298    |
| 6,156,118   | A    | 12/2000 | Silenius                              |
| 6,165,317   | A    | 12/2000 | Sabourin                              |
| 6,251,222   | B1   | 6/2001  | Silenius et al.                       |
| 6,296,736   | B1   | 10/2001 | Hsu et al.                            |
| 6,348,127   | B1   | 2/2002  | Gallagher et al.                      |
| 6,375,974   | B1   | 4/2002  | Ito et al.                            |
| 6,537,680   | B1   | 3/2003  | Norlander et al.                      |
| 6,599,391   | B2   | 7/2003  | Silenius et al.                       |
| 6,773,552   | B1   | 8/2004  | Albert et al.                         |
| 6,861,380   | B2   | 3/2005  | Garnier et al.                        |
| 6,887,350   | B2 * | 5/2005  | Garnier ..... D21H 13/10<br>162/146   |
| 6,935,589   | B1 * | 8/2005  | Matthew ..... D21D 1/306<br>241/261.3 |
| 6,946,058   | B2   | 9/2005  | Hu                                    |
| 6,955,309   | B2   | 10/2005 | Matthew et al.                        |
| 7,381,294   | B2   | 6/2008  | Suzuki et al.                         |
| 7,624,879   | B2   | 12/2009 | Frances                               |
| 7,741,234   | B2   | 6/2010  | Smith et al.                          |
| 7,942,964   | B2   | 5/2011  | Luo et al.                            |
| 8,419,899   | B2   | 4/2013  | Xia et al.                            |
| 8,871,057   | B2   | 10/2014 | Gane et al.                           |
| 9,297,112   | B2   | 3/2016  | Mesic et al.                          |
| 9,816,233   | B2   | 11/2017 | Shi et al.                            |
| 9,879,361   | B2   | 1/2018  | Pande et al.                          |
| 9,920,484   | B2 * | 3/2018  | Marcoccia ..... D21H 15/02            |
| 9,988,762   | B2 * | 6/2018  | Bilodeau ..... D21D 1/306             |
| 10,563,356  | B2   | 2/2020  | Marcoccia et al.                      |
| 10,704,165  | B2   | 7/2020  | Pande et al.                          |
| 10,710,930  | B2   | 7/2020  | Marcoccia et al.                      |
| 11,473,245  | B2 * | 10/2022 | Marcoccia ..... D21H 15/02            |
| 11,499,269  | B2   | 11/2022 | Pande et al.                          |
| 11,608,596  | B2 * | 3/2023  | Pande ..... D21H 23/56                |
| 002/0011317 | A1   | 1/2002  | Lee                                   |
| 002/0059886 | A1   | 5/2002  | Merkley et al.                        |
| 002/0069791 | A1   | 6/2002  | Merkley et al.                        |
| 002/0084046 | A1   | 7/2002  | Hsu et al.                            |

|              |     |         |                               |
|--------------|-----|---------|-------------------------------|
| 2003/0111197 | A1  | 6/2003  | Hu                            |
| 2004/0065419 | A1  | 4/2004  | Lasmarias et al.              |
| 2004/0112558 | A1  | 6/2004  | Garnier et al.                |
| 2004/0112997 | A1  | 6/2004  | Matthew et al.                |
| 2004/0149403 | A1  | 8/2004  | Rheims et al.                 |
| 2004/0180184 | A1  | 9/2004  | Fillion et al.                |
| 2004/0241350 | A1  | 12/2004 | Koga et al.                   |
| 2005/0145348 | A1  | 7/2005  | Lee                           |
| 2005/0194477 | A1  | 9/2005  | Suzuki                        |
| 2006/0006264 | A1  | 1/2006  | Sabourin et al.               |
| 2007/0164143 | A1  | 7/2007  | Sabourin et al.               |
| 2008/0148999 | A1  | 6/2008  | Luo et al.                    |
| 2008/0227161 | A1  | 9/2008  | Levie et al.                  |
| 2009/0145562 | A1  | 6/2009  | Nguyen                        |
| 2009/0145842 | A1  | 6/2009  | Frances                       |
| 2009/0162602 | A1  | 6/2009  | Cottier et al.                |
| 2009/0221812 | A1  | 9/2009  | Ankerfors et al.              |
| 2009/0266500 | A1  | 10/2009 | Schubert et al.               |
| 2010/0065236 | A1  | 3/2010  | Henriksson et al.             |
| 2010/0218908 | A1  | 9/2010  | Silénius et al.               |
| 2010/0288456 | A1  | 11/2010 | Westland et al.               |
| 2011/0088858 | A1* | 4/2011  | Polat .....                   |
|              |     |         | D21C 5/005<br>162/91          |
| 2011/0277947 | A1  | 11/2011 | Hua et al.                    |
| 2011/0314726 | A1  | 12/2011 | Jameel et al.                 |
| 2012/0007363 | A1  | 1/2012  | Wang                          |
| 2012/0012031 | A1  | 1/2012  | Husband et al.                |
| 2012/0241114 | A1  | 9/2012  | Axrup et al.                  |
| 2012/0277710 | A1  | 11/2012 | Marinelli et al.              |
| 2013/0071655 | A1  | 3/2013  | Zwick et al.                  |
| 2013/0202870 | A1  | 8/2013  | Malmborg et al.               |
| 2013/0209749 | A1  | 8/2013  | Myangiro et al.               |
| 2013/0248130 | A1  | 9/2013  | Stockhaus                     |
| 2014/0057105 | A1* | 2/2014  | Pande .....                   |
|              |     |         | D02J 3/02<br>428/401          |
| 2014/0116635 | A1  | 5/2014  | Porto et al.                  |
| 2014/0180184 | A1  | 6/2014  | Duguid                        |
| 2014/0209260 | A1  | 7/2014  | Li et al.                     |
| 2014/0209264 | A1  | 7/2014  | Tirimacco et al.              |
| 2014/0302117 | A1  | 10/2014 | Moen et al.                   |
| 2015/0299955 | A1  | 10/2015 | Laukkonen et al.              |
| 2016/0069029 | A1  | 3/2016  | Shannon                       |
| 2016/0138224 | A1  | 5/2016  | Shannon et al.                |
| 2016/0333524 | A1  | 11/2016 | Pande et al.                  |
| 2016/0340802 | A1  | 11/2016 | Pande et al.                  |
| 2017/0058457 | A1* | 3/2017  | Marcoccia .....               |
| 2017/0073893 | A1  | 3/2017  | D21H 11/16<br>Bilodeau et al. |
| 2017/0217654 | A1  | 8/2017  | Harmon                        |
| 2017/0226009 | A1  | 8/2017  | Marcoccia et al.              |
| 2017/0370036 | A1  | 12/2017 | Hermans et al.                |
| 2018/0105986 | A1  | 4/2018  | Pande et al.                  |
| 2018/0148895 | A1  | 5/2018  | Marcoccia et al.              |
| 2019/0218716 | A1  | 7/2019  | Hoglund et al.                |
| 2019/0242062 | A1* | 8/2019  | Harshad .....                 |
| 2020/0063353 | A1  | 2/2020  | Everett et al.                |
| 2020/0308769 | A1  | 10/2020 | Pande et al.                  |
| 2020/0325629 | A1  | 10/2020 | Marcoccia et al.              |
| 2020/0340155 | A1* | 10/2020 | Pande .....                   |
| 2021/0207289 | A1* | 7/2021  | Pande .....                   |
| 2022/0333312 | A1* | 10/2022 | Langford .....                |
| 2022/0333314 | A1* | 10/2022 | D21F 11/14<br>Langford .....  |
| 2022/0356648 | A1* | 11/2022 | D21H 17/71<br>Pande .....     |
| 2023/0035105 | A1* | 2/2023  | D21D 99/00<br>Marcoccia ..... |
| 2023/0084180 | A1  | 3/2023  | Pande et al.                  |
| 2023/0250588 | A1* | 8/2023  | Pande .....                   |
|              |     |         | D21C 5/02<br>162/149          |
| 2023/0366155 | A1* | 10/2023 | Zwick .....                   |
|              |     |         | D21H 27/38                    |

## FOREIGN PATENT DOCUMENTS

|    |           |      |         |                   |
|----|-----------|------|---------|-------------------|
| CA | 2883161   | A1   | 2/2014  |                   |
| CA | 3150203   | A1 * | 4/2021  | ..... D21C 9/007  |
| CN | 1516768   | A    | 7/2004  |                   |
| CN | 1718914   | A    | 1/2006  |                   |
| CN | 101691700 | A    | 4/2010  |                   |
| CN | 102971462 | A    | 3/2013  |                   |
| CN | 103590283 | B    | 12/2015 |                   |
| CN | 108867181 | A    | 11/2018 |                   |
| CN | 111788057 | B *  | 5/2022  | ..... B29C 43/003 |

(56)

## References Cited

## FOREIGN PATENT DOCUMENTS

EP 0333209 A2 9/1989  
 EP 0333212 A2 9/1989  
 EP 1232854 A1 8/2002  
 EP 2191066 A1 6/2010  
 EP 2220291 A1 8/2010  
 EP 2888401 B1 \* 1/2018 ..... D01B 9/00  
 EP 3108059 B1 \* 8/2019 ..... D21C 9/007  
 FR 2520769 A1 8/1983  
 JP S58136895 A 8/1983  
 JP H02229747 A 9/1990  
 JP H03122038 A 5/1991  
 JP H04194097 A 7/1992  
 JP H04263699 A 9/1992  
 JP H07165456 A 6/1995  
 JP H08197836 A 8/1996  
 JP H08284090 A 10/1996  
 JP H09124950 A 5/1997  
 JP 2002194691 A 7/2002  
 JP 2004525284 A 8/2004  
 JP 2004360088 A 12/2004  
 JP 2007231438 A 9/2007  
 JP 2010125694 A 6/2010  
 JP 2012526923 A 11/2012  
 JP 2015526608 A 9/2015  
 JP 2018135631 A 8/2018  
 KR 20040022874 A 3/2004  
 KR 10-20050086850 A 8/2005  
 KR 100662043 B1 12/2006  
 KR 10-2010-0090745 A 8/2010  
 KR 10-20130132381 A 12/2013  
 RU 2224060 C2 2/2004  
 RU 2309211 C2 10/2007  
 RU 2358055 C2 6/2009  
 WO 1996004424 A1 2/1996  
 WO 1998023814 A1 6/1998  
 WO 2002014606 A2 2/2002  
 WO 2002095129 A1 11/2002  
 WO 2004101889 A2 11/2004  
 WO 2009014483 A1 1/2009  
 WO 2009038730 A1 3/2009  
 WO 2009155541 A2 12/2009  
 WO 2010134868 A1 11/2010  
 WO 2012007363 A1 1/2012  
 WO 2012101331 A1 8/2012  
 WO 2014031737 A1 2/2014  
 WO 2014106684 A1 7/2014  
 WO 2015127233 A1 8/2015  
 WO 2015127239 A1 8/2015  
 WO WO-2017196519 A1 \* 11/2017 ..... A47K 10/16  
 WO 2018026804 A1 2/2018  
 WO 2018051275 A2 3/2018  
 WO 2019152969 A1 8/2019  
 WO WO-2021061723 A1 \* 4/2021 ..... D21C 9/007  
 WO WO-2021061747 A1 \* 4/2021 ..... D21D 1/34

## OTHER PUBLICATIONS

Applicant Initiated Interview Summary for U.S. Appl. No. 13/836,760, dated May 9, 2017.  
 Applicant Initiated Interview Summary for U.S. Appl. No. 13/836,760, dated Sep. 27, 2017.  
 Brazilian Notice of Rejection in corresponding Brazilian Patent Application No. 1120150038190 dated May 24, 2022 with English summary.  
 Brazilian Search Report issued in Corresponding Brazilian Patent Application No. BR112015003819-0, dated Sep. 9, 2019.  
 Carvalho, et al., "A Comparative Study for Two Automated Techniques for Measuring Fiber length," Tappi Journal, Technical Association of The Pulp & Paper Industry, 80(2): 137-142, 1997.  
 Declaration of Harshad Pande and Bruno Marcoccia, filed in U.S. Appl. No. 13/836,760, dated Oct. 12, 2016.  
 Demuner et al., "Ultra Low Intensity Refining of Eucalyptus Pulps." Scientific and Technical Advances in Refining and Mechanical Pulping 2005.

Extended European Search Report issued in European Application No. 17195921.6, mailed Nov. 20, 2017.  
 Final Office Action issued in U.S. Appl. No. 13/836,760, dated May 12, 2016.  
 Final Office Action issued in U.S. Appl. No. 13/838,760, dated Jan. 27, 2017.  
 Handbook of Pulping and Papermaking, C. Biermann, Academic Press; 2nd Edition (Aug. 5, 1996), p. 145.  
 Intention to grant for European Patent Application No. 13759601.1, dated Jul. 25, 2017, 45 pgs.  
 International Preliminary Report on Patentability for PCT Application No. PCT/US2013/055971, dated Feb. 24, 2015.  
 International Preliminary Report on Patentability issued in International Patent Application No. PCT/US2015/016858, dated Aug. 23, 2016.  
 International Preliminary Report on Patentability issued in International Patent Application No. PCT/US2015/016865, dated Aug. 23, 2016.  
 International Search Report and Written Opinion dated May 16, 2023 from International Application No. PCT/US2023/060044, International Filing Date Jan. 3, 2023.  
 International Search Report and Written Opinion for PCT Application No. PCT/US2013/055971, dated Oct. 24, 2013.  
 International Search Report and Written Opinion from International Application No. PCT/US2020/52179 dated Jan. 29, 2021, International Filing Date Sep. 23, 2020.  
 International Search Report and Written Opinion from International Application No. PCT/US2020/052138 dated Jan. 18, 2021, International Filing Date Sep. 23, 2020.  
 International Search Report and Written Opinion from International Application No. PCT/US2020/054470 dated May 2, 2021, International Filing Date Oct. 7, 2020.  
 International Search Report and Written Opinion issued in International Patent Application No. PCT/US2015/016858, dated May 15, 2015.  
 International Search Report and Written Opinion issued in International Patent Application No. PCT/US2015/016865, dated May 20, 2015.  
 International Search Report and written Opinion issued in International Patent Application No. PCT/US2017/044881, dated Oct. 18, 2017.  
 International Search Report and written Opinion issued in International Patent Application No. PCT/US2017/057161, dated Dec. 22, 2017.  
 International Search Report and written Opinion issued in International Patent Application No. PCT/US2019/016590, dated May 23, 2019.  
 International Search Report and written Opinion issued in International Patent Application No. PCT/US2020/025037, dated Jul. 16, 2020.  
 Joy et al., "Ultra-Low Intensity Refining of Short Fibered Pulps." African Pulp and Paper Week 2004 retrieved from URL :<
 Non-Final Office Action for U.S. Appl. No. 13/836,760, dated Oct. 15, 2015.  
 Notice of Acceptance for Australian Application No. 2013305802, dated Apr. 21, 2017.  
 Notice of Acceptance for New Zealand Application No. 705191, dated Apr. 13, 2017.  
 Notice of Allowance for Canadian Patent Application No. 2,883,161, Jan. 3, 2017.  
 Notice of Grant for Chinese Application No. 201380054919.2, mailed Nov. 14, 2017.  
 Notice of Reasons for Refusal issued in Japanese Patent Application No. 2018-090071, dated May 15, 2019.

(56)

**References Cited****OTHER PUBLICATIONS**

Office Action issued in Corresponding Chinese Patent Application No. 201810081469.0, dated Jan. 21, 2020.

Office Action issued in corresponding European Patent No. 17195921 dated Apr. 17, 2019.

Office Action Issued in Corresponding Korean Patent Application No. 10-2015-7006955, dated May 29, 2020.

Office Action issued in Indian Patent Application No. 465/KOLNP/2015, dated May 7, 2019.

Office Action issued in Russian Patent Application No. 2018125883/12, dated Mar. 6, 2019.

Pal et al., "A Simple Method for Calculation of the Permeability Coefficient of Porous Media," TAPPI Journal, 5(9):10-16, (2006).

Pala et al., "Refining and Enzymatic Treatment of Secondary Fibres for Paperboard Production: Cyberflex Measurements of Fibre Flexibility" Cost E20—Wood Fibre Cell Wall Structure 2001, 4 pages. Restriction Requirement for U.S. Appl. No. 13/836,760, dated Jul. 16, 2015.

Smook, Handbook for Pulp and Paper Technologists, 1992, Angus Wilde Publications, 2nd Edition, Chapters 13, 15, 16 and 20 (Year: 1992).

Teixeira, "Recycled Old Corrugated Container Fibers for Wood-Fiber Cement Sheets," International Scholarly Research Network 2012(923413): 1-8, 2012.

Tonoli et al., "Effect of Fibre morphology on flocculation of fibre-cement suspensions," Cement and Concrete Research, 39:1017-1022, (2009).

International Search Report and Written Opinion issued in International Application No. PCT/US2020/028986, dated Jul. 17, 2020. Liner International Paper, [www.Internationalpaper.com/products/asia/containerboard/product-detail/liner-ipad](http://www.Internationalpaper.com/products/asia/containerboard/product-detail/liner-ipad), downloaded on Aug. 3, 2021, 3 pgs., Year 2021.

Norton, Sarilee, Lightweight Containerboard in North America— "Can You Hear Me Now?", Jan./Feb. 2013, PaperAge, pp. 18-21 (Year 2013).

Notice of Allowance Issued in Chinese Patent Application No. 201580020488.7, dated Apr. 8, 2018.

Office Action issued in Japanese Application No. 2016-552985, dated Apr. 10, 2018.

Smook, Handbook for Pulp and Paper Technologists, 1992, Angus Wilde Publications, 2nd Edition, Chapter 9 (Year: 1992).

International Search Report and Written Opinion from corresponding International Application No. PCT/US2020/52146 dated Dec. 8, 2020, International Filing Date Sep. 23, 2020.

\* cited by examiner

**FIG. 1A****FIG. 1B**

**FIG. 2A****FIG. 2B****FIG. 3**

**FIG. 4A**



FIG. 4B



FIG. 4C

**TISSUES AND PAPER TOWELS  
INCORPORATING SURFACE ENHANCED  
PULP FIBERS AND METHODS OF MAKING  
THE SAME**

**CROSS-REFERENCE TO RELATED  
APPLICATIONS**

This application is a U.S. National Application of International Patent Application No. PCT/US2020/052146 filed Sep. 23, 2020 and claims priority to and the benefit of U.S. Provisional Application No. 62/904,397, filed Sep. 23, 2019, the contents of both of which are incorporated into the present application by references in their entirety.

**FIELD OF INVENTION**

The present invention relates generally to tissues and paper towels and, more particularly, to tissues and paper towels that incorporate surface enhanced pulp fibers.

**BACKGROUND**

Paper products such as, for example, tissues (e.g., bath and facial tissues), paper towels, and paper napkins, in general, desirably have high strength and softness. The final paper characteristics may involve compromises between different attributes that can result from constraints imposed by the fibers used to make the paper product. For example, strength and softness tend to be inversely related—increasing the proportion of strengthening fibers (e.g., softwood fibers) in the product may increase strength at the expense of softness. The product may have minimum strength requirements that, because of the inverse relationship between strength and softness, limit the product's achievable softness. To illustrate, the paper product may need to have an adequate basis weight to achieve suitable strength—conventional two-ply tissues may have a basis weight that is at least 45 grams per square meter (gsm) and conventional two-ply paper towels may have a basis weight that is at least 55 gsm.

Manufacturing considerations may also impose constraints on final paper characteristics. For example, while conventional fibrillated fibers may promote strength in a paper product, pulps including such fibers may have a low freeness, rendering them difficult to dry. Incorporating conventional fibrillated fibers into a furnish may thus increase papermaking costs (e.g., due to higher drying energy requirements). As such, the degree of fibrillation and/or the amount of fibrillated fibers incorporated into the product may be limited in prior art paper products such as tissues, paper towels, and paper napkins.

**SUMMARY**

There accordingly is a need in the art for paper products that can achieve a better combination of strength and softness than prior art products. The present paper products—which can include, without limitation, tissues (e.g., facial or bath tissues), paper towels, and paper napkins—address this need in the art by including surface enhanced pulp fibers (SEPF)—which can be highly fibrillated in a manner that significantly increases fiber surface area while mitigating reductions in fiber length—in addition to a plurality of unrefined or lightly fibrillated (compared to the SEPF) hardwood, softwood, and/or non-wood fibers. The paper product can comprise one or more plies (e.g., can be a single-ply or a multi-ply product) and can have a lower basis

weight than prior art products. For example, some of the present tissues can have a basis weight that is less than or equal to 21 gsm per ply. Such low basis weight products incorporating a combination of SEPF and unrefined or lightly fibrillated fibers can have a softness that is comparable to prior art products (e.g., a comparable stiffness and/or surface friction), but can also be stronger than those prior art products.

For some of the present paper products, at least one of (up to and including each of) the one or more plies can be a sheet having multiple layers arranged to promote softness (e.g., a soft surface feel). For example, at least one of the one or more plies can comprise one or more layers that comprise hardwood fibers—at least one of which defines an upper or lower surface of the paper product—and one or more layers that comprise the SEPF and softwood fibers. Because the hardwood fibers can promote tactile softness, positioning a hardwood fiber layer at the surface of the paper product can improve the tactile feel thereof, compared to products in which softwood fiber layers define the surface of the product.

The inclusion of SEPF can also reduce manufacturing costs. First, costs can be reduced at least in part because a product (e.g., a tissue, towel, or napkin) incorporating SEPF can achieve a better combination of strength and softness at a relatively low basis weight, which can reduce the amount of material required to form the product. And, unexpectedly, furnishes including SEPF can be easier to dry (e.g., in a through-air drying process) than otherwise comparable furnishes without SEPF, even though SEPF are highly fibrillated and have a high water retention value. This can reduce energy costs during the papermaking process.

Some of the present tissues comprise a first plurality of fibers that are hardwood fibers—which optionally comprise bleached eucalyptus fibers—and a second plurality of fibers. The second fibers, in some tissues, include surface enhanced pulp fibers (SEPF) and, optionally, softwood fibers, which optionally comprise norther bleached softwood kraft pulp (NBSK) fibers. In some embodiments, the SEPF are made by refining a pulp feed, the refining including for each of one or more refiners introducing the pulp feed between two refining elements of the refiner and rotating at least one of the refining elements, wherein refining the pulp feed is performed such that the refiner(s) consume at least 300 kilowatt-hours (kWh) per ton of fiber in the pulp feed. Each of the refining elements, in some embodiments, comprise a plurality of bars, each protruding from a surface of the refining element and having a width that is less than or equal to 1.3 millimeters (mm), and a plurality of grooves defined by the bars, each having a width that is less than or equal to 2.5 mm. The SEPF, in some tissues have a length weighted average fiber length that is at least 0.20 millimeters (mm), optionally at least 0.40 mm, and/or an average hydrodynamic specific surface area that is at least 10 square meters per gram (m<sup>2</sup>/g), optionally at least 12 m<sup>2</sup>/g. The SEPF, in some tissues, are softwood fibers. In some tissues, by weight between 50% and 80%—optionally between 65% and 75%—of the fibers of the tissue are the first fibers and/or at least 20%—optionally at least 25%—of the fibers of the tissue are the second fibers. In some tissues, by weight at least 90% of the second fibers are the softwood fibers and/or between 1% and 10% of the second fibers are the SEPF.

Some tissues include two or more fibers layers. The fiber layers, in some tissues, include one or more first fiber layers that comprise the first fibers, optionally where at least 90% of the fibers of the first fiber layer(s) are the first fibers, and one or more second fiber layers that comprise the second

fibers, optionally where at least 90% of the fibers of the second fiber layer(s) are the second fibers. At least one of the first fiber layer(s), in some tissues, defines one of opposing upper and lower surfaces of the tissue. In some tissues, the one or more first fiber layers comprise two first fiber layers, each defining a respective one of the upper and lower surfaces of the tissue and, optionally, each of the one or more second fiber layers disposed between the two first fiber layers. In some tissues, a total basis weight of the second fiber layer(s) is between 25% and 35% of the total basis weight of the first fiber layer(s).

Some tissues comprise one or more, optionally two or more, plies. In some tissues, the basis weight of the tissue is less than or equal to 21 grams per square meter (gsm) per ply.

For some tissues, a maximum cup crush load of the tissue is less than or equal to 1.0 Newton (N), optionally less than or equal to 1.06 N, and/or a tensile strength of the tissue is greater than or equal to 200 N/m, optionally greater than or equal to 220 N/m.

The term "coupled" is defined as connected, although not necessarily directly, and not necessarily mechanically; two items that are "coupled" may be unitary with each other. The terms "a" and "an" are defined as one or more unless this disclosure explicitly requires otherwise. The term "substantially" is defined as largely but not necessarily wholly what is specified—and includes what is specified; e.g., substantially 90 degrees includes 90 degrees and substantially parallel includes parallel—as understood by a person of ordinary skill in the art. In any disclosed embodiment, the terms "substantially" and "approximately" may be substituted with "within [a percentage] of" what is specified, where the percentage includes 0.1, 1, 5, and 10 percent.

The terms "comprise" and any form thereof such as "comprises" and "comprising," "have" and any form thereof such as "has" and "having," and "include" and any form thereof such as "includes" and "including" are open-ended linking verbs. As a result, a product or system that "comprises," "has," or "includes" one or more elements possesses those one or more elements, but is not limited to possessing only those elements. Likewise, a method that "comprises," "has," or "includes" one or more steps possesses those one or more steps, but is not limited to possessing only those one or more steps.

Any embodiment of any of the products, systems, and methods can consist of or consist essentially of—rather than comprise/include/have—any of the described steps, elements, and/or features. Thus, in any of the claims, the term "consisting of" or "consisting essentially of" can be substituted for any of the open-ended linking verbs recited above, in order to change the scope of a given claim from what it would otherwise be using the open-ended linking verb.

Further, a device or system that is configured in a certain way is configured in at least that way, but it can also be configured in other ways than those specifically described.

The feature or features of one embodiment may be applied to other embodiments, even though not described or illustrated, unless expressly prohibited by this disclosure or the nature of the embodiments.

Some details associated with the embodiments described above and others are described below.

#### BRIEF DESCRIPTION OF THE DRAWINGS

The following drawings illustrate by way of example and not limitation. For the sake of brevity and clarity, every feature of a given structure is not always labeled in every

figure in which that structure appears. Identical reference numbers do not necessarily indicate an identical structure. Rather, the same reference number may be used to indicate a similar feature or a feature with similar functionality, as may non-identical reference numbers.

FIG. 1A is a top view of a first embodiment of the present paper products.

FIG. 1B is a sectional view of the paper product of FIG. 1A taken along line 1B-1B and showing the layers thereof.

FIG. 2A is a schematic of a refining unit that can be used to produce surface enhanced pulp fibers. The refining unit of FIG. 2A includes a single refiner through which a pulp feed can be recirculated.

FIG. 2B is a schematic of another refining unit that can be used to produce surface enhanced pulp fibers. The refining unit of FIG. 2B includes two refiners, where a pulp feed can be recirculated through one of the refiners.

FIG. 3 is a schematic of two refining elements that can be used in the refiner(s) of FIGS. 2A and 2B to produce surface enhanced pulp fibers.

FIG. 4A is a schematic of a system that can be used to perform some of the present methods of making a paper product that comprises SEPF.

FIG. 4B is a schematic of a forming unit of the system of FIG. 4A that can be used to form one or more plies of one of the present paper products. As shown, the forming unit is configured for a through-air drying (TAD) process.

FIG. 4C is a schematic of a conversion unit of the system of FIG. 4A that can be used to laminate and/or emboss sheet(s) produced by the forming unit.

#### DETAILED DESCRIPTION

Referring to FIGS. 1A and 1B, shown is a paper product 10, which can be a tissue (e.g., a bath tissue or a facial tissue), a paper towel, or a paper napkin. Paper product 10 can comprise hardwood fibers (e.g., originating from oak, gum, maple, poplar, eucalyptus, aspen, birch, and/or the like), softwood fibers (e.g., originating from spruce, pine, fir, hemlock, redwood, and/or the like), and/or non-wood fibers (e.g., originating from kenaf, hemp, straws, bagasse, and/or the like), and, optionally, at least some of the fibers of the paper product can be recycled fibers. For example, paper product 10 can comprise a plurality of first fibers 14 that can be hardwood fibers—which can contribute to the softness of paper product 10—and a plurality of second fibers 18 that, to promote strength, can include softwood fibers 26 and a plurality of highly fibrillated fibers 30, referred to herein as "surface enhanced pulp fibers" (SEPF), that can be softwood fibers, hardwood fibers, or non-wood fibers. In other embodiments, however, the first and second fibers can comprise any suitable combination of fibers.

The non-SEPF fibers of paper product 10 (e.g., hardwood fibers 22 and softwood fibers 26) can be unrefined or lightly fibrillated (compared to SEPF 30)—those hardwood fibers and/or softwood fibers can have, for example, an average hydrodynamic specific surface area that is less than any one of, or between any two of, 3 square meters per gram ( $m^2/g$ ), 2.5  $m^2/g$ , 2  $m^2/g$ , 1.5  $m^2/g$ , or 1  $m^2/g$  (e.g., less than 2  $m^2/g$ ). SEPF 30 can have higher surface areas compared to conventionally-refined fibers, and can be made in a manner that mitigates reductions in fiber length that occur in conventional refining processes. For example, SEPF 30 can be made by refining a pulp feed (e.g., 34) with one or more mechanical refiners (e.g., 38a and/or 38b) (FIGS. 2A and 2B). Referring additionally to FIG. 3, each of the refiner(s) can comprise at least two refining elements (e.g., 42), each

including a plurality of bars (e.g., 50) that extend outwardly from a surface (e.g., 46) of the refining element and define a plurality of grooves (e.g., 54). For example, each of the refiner(s) can be a disk refiner (e.g., a single-disk refiner, a double-disk refiner, or a multi-disk refiner) (e.g., in which the refining elements are refiner plates) or a conical refiner (e.g., in which the refining elements are conical refiner fillings).

The pulp feed can be refined at least by, for each of the refiner(s), introducing the pulp feed between the refining elements and rotating at least one, optionally each, of the refining elements. The bars can thereby impart compression and shearing forces on the fibers of the pulp feed to increase the fibrillation, and thus the average hydrodynamic specific surface area, thereof. To facilitate a high degree of fibrillation while mitigating undesired reductions in fiber length, each of the refining elements can have a fine bar pattern and, optionally, the refiner(s) can be operated at a low intensity (e.g., at a low specific edge load (SEL)), compared to conventional refining processes. For example, for each of the refining elements, each of the bars can have a width (e.g., 58) that is less than or equal to any one of, or between any two of, 1.3 millimeters (mm), 1.2 mm, 1.1 mm, 1.0 mm, 0.9 mm, or 0.8 mm (e.g., less than or equal to 1.3 mm or 1.0 mm) and each of the grooves can have a width (e.g., 62) that is less than or equal to any one of, or between any two of, 2.5 mm, 2.3 mm, 2.1 mm, 1.9 mm, 1.7 mm, 1.5 mm, or 1.3 mm (e.g., less than or equal to 2.5 mm, 1.6 mm, or 1.3 mm). And, refining the pulp feed can be performed such that each of the refiner(s) operates at a SEL that is less than or equal to any one of, or between any two of, 0.70 Watt-seconds per meter (W·s/m), 0.60 W·s/m, 0.50 W·s/m, 0.40 W·s/m, 0.30 W·s/m, 0.25 W·s/m, 0.20 W·s/m, 0.15 W·s/m, or 0.10 W·s/m (e.g., between 0.1 and 0.3 W·s/m or 0.1 and 0.2 W·s/m).

The pulp feed can be refined using a large amount of refining energy, compared to conventional processes, to achieve a high degree of fibrillation. For example, refining the pulp feed can be performed such that, per ton of fiber in the pulp feed, the refiner(s) consume greater than or equal to any one of, or between any two of, 300 kilowatt-hours (kWh), 400 kWh, 500 kWh, 600 kWh, 700 kWh, 800 kWh, 900 kWh, or 1,000 kWh (e.g., greater than or equal to 300 kWh or 650 kWh per ton of fiber in the pulp feed). The refining energy expended can depend at least in part on the type of fibers in the pulp feed and the desired degree of fibrillation. Without limitation, when the pulp feed includes hardwood fibers, the refining energy can be between 300 and 650 kWh per ton of fiber and when the pulp feed includes softwood fibers, the refining energy can be at least 650 kWh, optionally at least 1,000 kWh, per ton of fiber (e.g., because softwood fibers, which are typically longer than hardwood fibers, may be subjected to more refining than hardwood fibers before fiber shortening and fines production adversely affects fiber quality).

Such refining energies can be reached in any suitable manner. For example, each of the refiner(s) can consume, per ton of fiber in the pulp feed, less than or equal to any one of, or between any two of, 110 kWh, 100 kWh, 90 kWh, 80 kWh, 70 kWh, 60 kWh, 50 kWh, 40 kWh, or 30 kWh each time the pulp feed is passed through the refiner. To reach the total desired refining energy, the pulp feed can be recirculated through at least one of the refiner(s) and/or passed through multiple refiners such that the cumulative energy consumed by the refiner(s) reaches the desired level (e.g., at least 300 kWh or 650 kWh per ton of fiber). Referring to FIG. 2A, for example, the one or more refiners can consist of a single refiner (e.g., 30a) (e.g., where, for each of the refiner's refining elements, each of the bars has a width that

is less than or equal to 1.3 mm and each of the grooves has a width that is less than or equal to 1.6 mm) and the pulp feed can be passed through the refiner a plurality of times (e.g., greater than or equal to any one of, or between any two of, 2, 6, 10, 14, 18, 22, or 26 times) until the refiner consumes the desired refining energy. Alternatively, and referring to FIG. 2B, the one or more refiners can comprise one or more first refiners (e.g., 30a) (e.g., a single first refiner) and one or more second refiners (e.g., 30b) such that the pulp feed passes through multiple refiners. Each of the first refiner(s) can be configured to fibrillate the fibers of the pulp feed with less refinement than the second refiner(s). For example, for each of the first refiner(s), each of the bars can have a width that is greater than or equal to 1.0 mm, each of the grooves can have a width that is greater than or equal 1.6 mm, and the first refiner can operate at a SEL between 0.2 and 0.3 W·s/m. The pulp feed can be introduced into the second refiner(s) after passing through the first refiner(s) and, for each of the second refiner(s), each of the bars can have a width that is less than or equal to 1.0 mm, each of the grooves can have a width that is less than or equal to 1.6 mm, and the second refiner can operate at a SEL between 0.1 and 0.2 W·s/m. The pulp feed can be recirculated through at least one of the second refiner(s) (e.g., as described with respect to FIG. 2A).

Such high-energy refining (e.g., at least 300 kWh per ton of fiber) performed using refining elements having a fine bar pattern (e.g., any of those described above) and/or at low intensity (e.g., at a SEL between 0.1 and 0.3 W·s/m) can yield larger increases in the average hydrodynamic specific area of the fibers of the pulp feed than conventional refining processes while mitigating reductions in fiber length. For example, the pulp feed can be refined such that the average hydrodynamic specific surface area of the pulp fibers increases by at least 300% (e.g., at least 700%) while the length weighted average fiber length of the fibers decreases by less than 30%. To illustrate, SEPF 30 can have a length weighted average fiber length that is greater than or equal to any one of, or between any two of, 0.20 millimeters (mm), 0.30 mm, 0.40 mm, 0.50 mm, 0.60 mm, 0.70 mm, 0.80 mm, 0.90 mm, 1.0 mm, 1.5 mm, or 2.0 mm (e.g., greater than or equal to 0.20 mm, 0.30 mm, or 0.40 mm or between 1.0 mm and 2.0 mm), and an average hydrodynamic specific surface area that is greater than or equal to any one of, or between any two of, 10 square meters per gram (m<sup>2</sup>/g), 12 m<sup>2</sup>/g, 14 m<sup>2</sup>/g, 16 m<sup>2</sup>/g, 18 m<sup>2</sup>/g, 20 m<sup>2</sup>/g, or larger (e.g., greater than or equal to 10 m<sup>2</sup>/g). Optionally, the number of SEPF can be at least 12,000 per milligram on an oven-dry basis (e.g., based on a sample of the SEPF that is dried in an oven set at 105° C. for 24 hours). A description of SEPF and processes by which SEPF can be made are set forth in further detail in U.S. patent application Ser. No. 13/836,760, filed Mar. 15, 2013, and published as Pub. No. US 2014/0057105 on Feb. 27, 2014, which is hereby incorporated by reference.

First fibers 14 and second fibers 18 can be obtained from any suitable process, such as, for example, a chemical process (e.g., a kraft process), a mechanical process, a thermomechanical process, a chemi-thermomechanical process, a recycling process, and/or the like, and can be bleached or unbleached. For example, softwood fibers 26 and/or SEPF 30 can be northern bleached softwood kraft (NBSK) pulp fibers and/or hardwood fibers 22 can be bleached eucalyptus (BEK) fibers; in other embodiments, however, the hardwood fibers, softwood fibers, and SEPF can be of any suitable type or combination of types. Paper product 10 can also, but need not, comprise a plurality of

third fibers that can be softwood fibers of a different grade (e.g., southern bleached softwood kraft (SBSK) pulp fibers) than softwood fibers **26** of second fibers **18**; the third fibers can also strengthen the paper product. Incorporating such fiber types in paper product **10** can yield a desired combination of strength and softness.

Any suitable proportion of first fibers **14** and second fibers **18** can be incorporated into paper product **10** to impart a suitable strength and softness thereon. Strength (e.g., wet and/or dry tensile strength) can be positively correlated with the proportion of second fibers **18** (e.g., softwood fibers **26** and SEPF **30**) in paper product **10**, while softness (e.g., related to stiffness and/or surface friction) can be positively correlated with the proportion of first fibers **14** (e.g., hardwood fibers **22**) in the paper product. As such, when paper product **10** is a product that is preferably relatively soft—such as a bath tissue—at least a majority of the fibers of the product can be first fibers **14**, e.g., by weight, greater than or equal to any one of, or between any two of, 50%, 60%, 70%, 80%, or 90% of the fibers of the product can be the first fibers (e.g., hardwood fibers **22**) and less than or equal to any one of, or between any two of, 40%, 30%, 20%, or 10% of the fibers of the product can be second fibers **18** (e.g., softwood fibers **26** and SEPF **30**). When paper product **10** is a product that preferably has a relatively high wet strength—such as a paper towel—a minority of the fibers of the paper product can be first fibers **14**, e.g., by weight, less than or equal to any one of, or between any two of, 40%, 30%, 20%, or 10% of the fibers of the paper product can be first fibers **14** (e.g., hardwood fibers **22**) and greater than or equal to any one of, or between any two of, 40%, 50%, 60%, 70%, 80%, or 90% of the fibers of the paper product can be second fibers **18** (e.g., softwood fibers **26** and SEPF **30**). Paper product **10**, when including the third fibers, can have more second fibers **18** than third fibers. For example, when paper product **10** is a paper towel, by weight, greater than or equal to any one of, or between any two of, 35%, 40%, 45%, 50%, 55%, 60%, or 65% of the fibers of the paper towel can be second fibers **18** and greater than or equal to any one of, or between any two of, 10%, 15%, 20%, 25%, or 30% of the fibers of the paper towel can be the third fibers.

These relationships between strength, softness, and the proportions of first fibers **14** and second fibers **18** in paper product **10** may not be monotonic, at least when the second fibers include SEPF **30**. For example, increasing the proportion of first fibers **14** (e.g., hardwood fibers **22**) in paper product **10** may improve softness up to a point, after which doing so may not yield an improvement in softness and can reduce strength, a sub-optimal result. First fibers **14** and second fibers **18** can be incorporated into paper product **10** in proportions that avoid such a sub-optimal combination of strength and softness. For example, when paper product **10** is a tissue, by weight between 50% and 80% (e.g., between 65% and 75%) of the tissue's fibers can be first fibers **14** and at least 20% (e.g., at least 25%) of the tissue's fibers can be second fibers **18**. And, when paper product **10** is a paper towel, by weight between 10% and 35% (e.g., between 15% and 25%) of the paper towel's fibers can be first fibers **14** and at least 40% (e.g., at least 50%) of the paper towel's fibers can be second fibers **18**. Optionally, when paper product **10** includes the third fibers, between 15% and 35% of the product's fibers can be the third fibers (e.g., softwood fibers of a different grade than softwood fibers **26**).

Paper product **10**, when comprising such proportions of first fibers **14** and second fibers **18**, can be stronger than otherwise similar products that do not comprise SEPF **30**. Such enhanced strength can be achieved when at least a

majority of second fibers **14** are softwood fibers **26**, e.g., by weight, greater than or equal to any one of, or between any two of, 50%, 60%, 70%, 80%, or 90% (e.g., at least 90%) of the second fibers can be the softwood fibers while less than or equal to any one of, or between any two of, 40%, 30%, 20%, 10%, or 5% (e.g., between 1% and 10%) of the second fibers can be SEPF **30**. The inclusion of SEPF **30** into paper product **10** can yield higher strengths (e.g., dry and/or wet tensile strengths) than otherwise comparable products at least in part because of the comparatively long fiber lengths and high surface areas of the SEPF. The large hydrodynamic specific surface area of SEPF **30**, for example, can promote chemical bonding and accommodate larger amounts of wet strength resins.

While the strength imparted by SEPF **30** may tend to decrease the softness of paper product **10** (e.g., by increasing stiffness), the paper product can nonetheless be stronger than prior art products at a given softness, an unexpected result. Such an improved combination of strength and softness may be achievable when paper product **10** has a basis weight that is lower than that of prior art paper products (e.g., prior art tissues, paper towels, and paper napkins) to promote softness. For example, paper product **10** can have a basis weight per ply (e.g., the total basis weight of the paper product divided by the number of plies thereof) that, when a tissue, is less than or equal to any one of, or between any two of, 22 grams per square meter (gsm), 21 gsm, 20 gsm, 19 gsm, 18 gsm, or 17 gsm (e.g., less than or equal to 21 gsm per ply) and, when a paper towel, is less than or equal to any one of, or between any two of, 26 gsm, 25 gsm, 24 gsm, 23 gsm, 22 gsm, or 21 gsm (e.g., less than or equal to 26 gsm per ply). Paper product **10**, when having such basis weights in combination with the above-described proportions of hardwood fibers **22**, softwood fibers **26**, and SEPF **30**, can have a desired softness for its intended application (e.g., comparable to or better than prior art products that are not as strong) while still exhibiting enhanced strength (e.g., attributable at least in part to SEPF **30**). To illustrate, when paper product **10** is a tissue, the tissue can have a dry tensile strength (e.g., in the machine and/or cross directions) that is greater than or equal to any one of, or between any two of, 200 Newtons per meter (N/m), 210 N/m, 220 N/m, 230 N/m, 240 N/m, 250 N/m, 260 N/m, or 270 N/m (e.g., greater than or equal to 200 N/m or 220 N/m) and a maximum cup crush load that is less than or equal to any one of, or between any two of, 1.06 N, 1.04 N, 1.02 N, 1.0 N, 0.95 N, 0.90 N, or 0.85 N (e.g., less than or equal to 1.06 N or 1.0 N). As used herein, maximum cup crush load can be measured pursuant to NWSP 402.0, *Cup Crush*, which is hereby incorporated by reference.

Paper product **10** can comprise one or more, optionally two or more, plies **32** (e.g., the paper product can be a single-ply or a multi-ply tissue or paper towel), each of which can comprise a single fiber layer or two or more fiber layers (e.g., **66a** and **66b**). When paper product **10** includes multiple fiber layers (e.g., by having at least one multi-layer ply or multiple single- and/or multi-layer plies), those layers can be arranged to promote softness. To illustrate, the fiber layers can include one or more first fiber layers **66a** that comprise first fibers **14** (e.g., hardwood fibers **22**) (e.g., such that at least 90% of the fibers of the first fiber layer(s) are the first fibers) and one or more second fiber layers **66b** that comprise second fibers **18** (e.g., softwood fibers **26** and SEPF **30**) (e.g., such that at least 90% of the fibers of the second fiber layer(s) are the second fibers). As such, first fiber layer(s) **66a** can be softer (e.g., have a softer tactile feel) than second fiber layer(s) **66b**, and the second fiber

layer(s) can provide comparatively more strength for paper product **10**. To achieve a soft tactile feel, at least one of first fiber layer(s) **66a** can define one of opposing upper and lower surfaces **70a** and **70b** of paper product **10**. As shown, for example, paper product **10** has two first fiber layers **66a**, each defining a respective one of upper and lower surfaces **70a** and **70b**, and one second fiber layer **66b** that is disposed between the first fiber layers, where all of the fiber layers are part of a single ply **32**. In other embodiments, however, paper product **10** can have any combination of single-layered and/or multi-layered plies arranged to achieve a desired layer positioning.

Fiber layers **66a** and **66b** can have any suitable basis weights to yield the above-described proportions of first fibers **14** and second fibers **18**. For example, the total basis weight of second fiber layer(s) **66b** can be less than or equal to any one of, or between any two of, 90%, 80%, 70%, 60%, 50%, 40%, 30%, or 20% (e.g., between 25% and 35%) of the total basis weight of first fiber layer(s) **66a**, when paper product **10** is a tissue.

Paper product **10** can be made in any suitable manner such as, for example, in a through-air drying ("TAD") process or a dry creping process. Referring to FIGS. **4A-4C**, shown is a system **74** that can be used to perform some of the present methods. While some methods are described with reference to system **74**, system **74** is not limiting on those methods, which can be performed using any suitable system. As an illustration, such suitable systems can include—but are not limited to—VALMET®'s ADVANTAGE™ QRT®, eTAD™, and NTT® systems and VOITH®'s ATMOS® system.

Some methods of making a paper product (e.g., a tissue, paper towel, or paper napkin) can include a step of making one or more sheets (e.g., **32**), each of which—as explained below—can define a respective ply of the paper product. Each of the sheet(s) can be made using one or more furnishes (e.g., **78a** and **78b**) (FIGS. **4A** and **4B**). The furnish(es) can comprise fibers (e.g., cellulosic fibers) dispersed in water, which can include any of the fibers discussed above, such as, for example, a plurality of first fibers (e.g., **14**) that can be hardwood fibers (e.g., **22**), a plurality of second fibers (e.g., **18**) that can include softwood fibers (e.g., **26**) and SEPF (e.g., **30**), and, optionally, a plurality of third fibers that can be softwood fibers of a different grade than those of the second fibers.

To illustrate, the furnish(es) can comprise a first furnish (e.g., **78a**) and a second furnish (e.g., **78b**). The first furnish can comprise the first fibers and, optionally, the third fibers (e.g., such that at least 90% of the fibers of the first furnish, by weight, are the first and, optionally, third fibers). The second furnish can comprise the second fibers (e.g., such that at least 90% of the fibers of the second furnish, by weight, are the second fibers). In other embodiments, however, the fibers can be distributed amongst any suitable number of furnishes in any suitable manner.

The relative proportions of first, second, and third fibers in the furnish(es) can be such that the paper product, when made, has any of the above-described proportions of fibers. As an example, for each of the sheet(s), the furnish(es) can include any of the proportions of first, second, and third fibers discussed above with respect to paper product **10**—when making a tissue, between 50% and 80% of the fibers of the furnish(es) can be the first fibers and at least 20% of the fibers of the furnish(es) can be the second fibers. And, when making a paper towel, between 10% and 35% of the fibers of the furnish(es) can be the first fibers, at least 40% of the fibers of the furnish(es) can be the second fibers,

and, optionally, between 15% and 35% of the fibers of the furnish(es) can be the third fibers.

Some methods include a step of introducing one or more wet strength resins to the furnish(es). The wet strength resin(s) can include any suitable resins, such as, for example, one or more cationic wet strength resins, and can be permanent or temporary. To illustrate, the wet strength resin(s) can comprise polyamide-epichlorohydrin (PAE) and/or carboxymethyl cellulose (e.g., when making a paper towel) or a polyacrylamide resin (e.g., when making a tissue). Other suitable wet strength resins can include urea formaldehyde resins, melamine formaldehyde resins, polythylenimine resins, and/or the like. Yet further suitable wet strength resins are set forth in Wet Strength in Paper and Paperboard, TAPPI Monograph Series No. 29 (Technical Association of the Pulp and Paper Industry, New York, 1965), which is hereby incorporated by reference. The wet strength resin(s) can promote wet strength in the formed paper product, and can be added in any suitable amounts to achieve a desired wet strength. For example, when making a paper towel, introducing the wet strength resin(s) can be performed such that, per ton of fiber in the furnish(es), greater than or equal to any one of, or between any two of, 6 kilograms (kg), 7 kg, 8 kg, 9 kg, 10 kg, 11 kg, 12 kg, 13 kg, 14 kg, 15 kg, 16 kg, 17 kg, or 18 kg (e.g., greater than or equal to 12 or 13 kg) of PAE are introduced and/or greater than or equal to any one of, or between any two of, 1.8 kg, 1.9 kg, 2.0 kg, 2.1 kg, 2.2 kg, 2.3 kg, 2.4 kg, 2.5 kg, 2.6 kg, 2.7 kg, or 2.8 kg (e.g., greater than or equal to 2.5 kg) of carboxymethyl cellulose are introduced. When making a tissue, greater than or equal to any one of, or between any two of, 0.8 kg, 0.9 kg, 1.0 kg, 1.1 kg, or 1.2 kg (e.g., greater than or equal to 0.9 kg) of a polyacrylamide resin (e.g., a glyoxalated cationic polyacrylamide resin) can be introduced. In prior art methods, the amount of wet strength resin(s) retainable by conventional fibers is limited; SEPF can retain more chemicals than conventional fibers and, as such, the above-described amounts of wet strength resin(s) may be higher than those used in prior art methods.

Some methods comprise a step of refining at least some of the furnish(es) with one or more refiners (e.g., **82**). For example, as shown the second furnish can be beaten with one or more mechanical refiners to fibrillate (or further fibrillate) the softwood fibers and/or SEPF. Each of the mechanical refiner(s) can be any suitable refiner, such as, for example, a double disk refiner, a conical refiner, a single disk refiner, a multi-disk refiner, a conical refiner, and/or the like. The second furnish can also be refined chemically in addition to or instead of mechanical refining, such as with one or more enzymes (e.g., cellulases and/or xylanases). Refining can be performed such that the second furnish reaches a freeness that is less than or equal to any one of, or between any two of, 620 ml CSF, 600 ml CSF, 580 ml CSF, 560 ml CSF, 540 ml CSF, 520 ml CSF, 500 ml CSF, 480 ml CSF, 460 ml CSF, 440 ml CSF, 420 ml CSF, 400 ml CSF, 380 ml CSF, or 360 ml CSF (e.g., less than or equal to 450 ml CSF, for tissue, or less than or equal to 620 ml CSF, for towel). The presence of SEPF in the second furnish may reduce the refining energy required to achieve a desired freeness, and thus strength, compared to conventional processes. For example, in some methods beating the second furnish can be performed until the refiner(s) consume less than or equal to 40 kWh (e.g., between 25 and 40 kWh) (e.g., if the paper product is a tissue) or less than or equal to 30 kWh (e.g., between 20 and 30 kWh) (e.g., if the paper product is a paper towel) per ton of fiber in the second furnish. The first furnish, in some methods, is not refined (which may, at least in some

## 11

instances, preserve the fiber length of the hardwood fibers thereof). Such selective refining of furnishes can facilitate production of a paper product having a combination of strength and softness that is better than that of prior art products.

The sheet(s) can be made in one or more forming units (e.g., 86) (FIG. 4B). For each of the sheet(s), some methods comprise a step of forming a web (e.g., 90) at least by depositing the furnish(es) onto one or more moving surface(s) (e.g., 94a and 94b) (e.g., with one or more, optionally two or more, head boxes (e.g., 98)). For example, the forming unit can comprise a twin-wire former including two wires (e.g., 102a and 102b) and the furnish(es) can be deposited onto and/or between the moving surfaces of the wires. Any suitable combination of the furnish(es) can be used to form the web. For example, the first furnish and the refined second furnish can be combined and the web can be formed from at least the combined first and second furnishes (e.g., such that the web, and thus the sheet, comprises a single layer). In other embodiments, however, the furnish(es) can be deposited onto the moving surface(s) to form a multi-layered web and, thus, sheet (e.g., by depositing the furnish(es) with a single headbox and using leaves to divide the deposited furnish(es) into layers, which may be suitable for low-basis weight products like tissues, or by using multiple head boxes, each configured to form one of the fiber layers). To illustrate, the furnish(es) can be deposited such that the web, and thus sheet, includes one or more first fiber layers (e.g., formed from the first furnish, optionally such that at least 90% of the fibers of the first fiber layer(s), by weight, are the first fibers and/or third fibers) and one or more second fiber layers (e.g., formed from the second furnish). The layers can be formed such that the web, and thus the sheet, has the arrangement of fiber layers shown in FIG. 1B. The furnish(es) can be deposited such that the web has any of the above described proportions of first fibers, second fibers, and, optionally, third fibers.

Some methods comprise a step of at least partially dewatering the web to form the sheet. The web can be at least partially dewatered at least by drawing water from the web with one or more vacuums (e.g., 106) (e.g., while the web is disposed on at least one of the moving surface(s)). Dewatering can also, but need not, be achieved in a TAD process. For example, as shown, the web can be transferred to a fabric (e.g., 110) (e.g., a woven fabric, which can provide three-dimensional structure for the web) and passed partially around each of one or more—optionally two or more—TAD rolls (e.g., 114) and, while being passed partially around the TAD roll(s), a gas (e.g., air) can be directed through the web. The gas can be heated to facilitate drying. This can be done, for example, by burning a fuel such as a combustible gas (e.g., natural gas) to heat air. The web can also be passed partially around a Yankee dryer (e.g., 118), which can be a heated vessel. The Yankee dryer can be heated using steam, which may be directed into the vessel where the steam can transfer heat to the outer surface thereof, condense, and be collected.

While SEPF can have a higher water retention value (WRV) than unfibrillated or lightly fibrillated fibers, the inclusion of SEPF in the web can unexpectedly facilitate drying (e.g., by reducing fuel and/or steam requirements for the TAD roll(s) and Yankee dryer, respectively), particularly when the basis weight of the web is comparatively low. For at least some paper towels, to achieve a suitable level of drying, the total flow of fuel (e.g., natural gas) to heat the gas (e.g., air) for all (e.g., two) TAD roll(s) can be less than or equal to any one of, or between any two of, 223 kg/hr, 221

## 12

kg/hr, 219 kg/hr, 217 kg/hr, 215 kg/hr, or 213 kg/hr. This may be at least 7% lower than that required for a web that does not include SEPF. And, the flow of steam for the Yankee dryer can be less than or equal to any one of, or between any two of, 1020 kg/hr, 1010 kg/r, 1000 kg/hr, 990 kg/hr, 980 kg/r, 970 kg/hr, or 960 kg/hr, which may similarly be at least 7% lower than that required for SEPF-free webs. For at least some tissues, the fuel (e.g., natural gas) flow rate for the TAD roll(s) can be less than or equal to any one of, or between any two of, 185 kg/hr, 183 kg/hr, 181 kg/hr, 179 kg/hr, 177 kg/hr, 175 kg/hr, or 173 kg/or, and/or the steam flow rate for the Yankee dryer can be less than or equal to any one of, or between any two of, 1035 kg/hr, 1025 kg/hr, 1015 kg/hr, 1005 kg/hr, 995 kg/hr, 985 kg/hr, 975 kg/hr, 965 kg/hr, 955 kg/r, 945 kg/hr, or 935 kg/hr. These fuel and steam flow rates may be at least 9% and 5% smaller, respectively, than those required for SEPF-free webs.

The surface of the Yankee dryer can be coated with a polymer (e.g., adhesive) that can facilitate retention of the web on the Yankee dryer. A creeping blade can be configured to remove the web from the Yankee dryer and/or can crepe the web. The coating deposited on the Yankee dryer's surface can include a releasing agent to facilitate this removal. The formed sheet can be wound onto a reel (e.g., 122) to form a roll. Such a TAD process can promote high bulk in the paper product to achieve lower basis weights; however, in other embodiments, any suitable forming process can be used to make the sheet(s).

One or more—optionally two or more—sheets can be formed as described above. Some methods comprise a step of embossing the sheet(s) and/or—if multiple sheets are produced—laminating the sheets in a conversion unit (e.g., 126) (FIG. 4C). Each of the sheet(s) can define a respective ply of the paper product (e.g., 10). For example, to make a multi-ply paper product, if each of the sheets is wound onto a reel, the rolls can be unwound and the sheets can be layered. The layered sheets can be embossed with an embosser (e.g., 130) that, optionally, comprises two or more pressing elements (e.g., 134a and 134b) (e.g., two or more rollers). The layered sheets can be passed between the pressing elements, at least one of which can comprise a plurality of protrusions (e.g., 138) such that the sheets are embossed. The embossing and laminating can be performed simultaneously, e.g., the embossing can cause and/or facilitate bonding of the sheets. However, in other embodiments, lamination can be performed in any suitable manner, such as, for example, by applying an adhesive, ultrasonic bonds, and/or the like. Laminating and embossing may also be performed separately, e.g., the sheets can be embossed after lamination and/or at least one of the sheets can be embossed prior to lamination. While as shown multiple sheets are laminated to form a multi-ply paper product (e.g., having two or more plies), in other embodiments a single-ply paper product can be formed from a single sheet (e.g., with no lamination, whether or not the single sheet is embossed).

Forming, laminating, and/or embossing the sheet(s) can be performed such that the paper product has any of the basis weights described above with respect to paper product 10. The basis weight of each of the sheet(s) may be lower than the per ply basis weight of the paper product, at least for some multi-ply paper products where the laminating process can increase the weight thereof. Additionally, forming and/or laminating the sheet(s) can be performed such that the paper product has any of the above-described arrangements of fiber layers (e.g., to promote softness).

The paper product can be subject to one or more processes after lamination and/or embossing to prepare the product for

market. For example, the produced paper product (e.g., a paper towel or bath tissue) can be rolled onto one or more reels (e.g., 142). When multiple reels are used, for at least one of the reels the paper product can be cut (e.g., with a cutter 146) after rolling a portion of the paper product onto the reel (e.g., to separate the portion of the paper product and thereby form a roll of a desired size). Other packaging techniques can be used as well. For example, when the paper product is a facial tissue, cut portions of the tissue can be folded and/or packaged in a box.

## EXAMPLES

The present invention will be described in greater detail by way of specific examples. The following examples are offered for illustrative purposes only and are not intended to limit the present invention in any manner. Those skilled in the art will readily recognize a variety of non-critical parameters that can be changed or modified to yield essentially the same results.

## Example 1

Six two-ply tissue samples were made using a TAD process: three where each of the plies had multiple layers (Tissue Samples 1-3) and six where each of the plies had a single layer (Tissue Samples 4-9). Each of the samples comprised first fibers that were BEK fibers and second fibers that included NBSK fibers and softwood SEPF. When making each of the samples, the first fibers were part of a first furnish and the second fibers were part of a second furnish that was beaten with a mechanical refiner. One kilogram of HERCOBOND™ 1194 dry strength resin per ton of fiber was introduced into the furnishes. For single-layer samples, each of the plies was made by combining the first furnish and beaten second furnish and using the furnishes to form a web. For multi-layer samples, each of the plies was made by forming a web with the first furnish and beaten second furnish such that the beaten second furnish formed a layer disposed between two layers formed from the first furnish. The web was dewatered using vacuums and through-air drying. The TAD system included two TAD rolls and a Yankee dryer—the air used for each of the TAD rolls was heated by burning propane and the Yankee dryer was heated with steam (e.g., as described above). For all samples, two plies were produced and laminated to make a two-ply tissue.

The proportions of first and second fibers, refining energy, and basis weight were varied and tissue properties—including caliper, bulk, cup crush load and energy (e.g., pursuant to NWS 402.0, *Cup Crush*), burst strength, and machine direction and cross-direction tensile strength, stretch, and tensile energy absorption (TEA)—were measured. Tissue Samples 1 and 4 were used as controls—those samples did not include SEPF, while in the other samples 10% of the second fibers, by weight, were SEPF. TABLES 1 and 2 sets forth the results for the multi-layer and single-layers tissues, respectively.

TABLE 1

|    |                                  | Properties of Multi-Layer Tissues |        |        |
|----|----------------------------------|-----------------------------------|--------|--------|
|    |                                  | Tissue Sample                     |        |        |
|    |                                  | 1                                 | 2      | 3      |
| 20 | First Fibers (% tissue fibers)   | 70                                | 70     | 70     |
|    | Second Fibers (% tissue fibers)  | 30                                | 30     | 30     |
|    | SEPF (% of second fibers)        | 0                                 | 10     | 10     |
| 25 | Refining Energy (kWh/t)          | 62.3                              | 59.3   | 20.7   |
|    | TAD Roll 1 Propane Flow (kg/hr)  | 117                               | 113    | 124    |
|    | TAD Roll 2 Propane Flow (kg/hr)  | 70.1                              | 71.8   | 76     |
| 30 | Total TAD Propane Flow (kg/hr)   | 187.1                             | 184.8  | 200    |
|    | Yankee Dryer Steam Flow (kg/hr)  | 1050                              | 1091   | 1041   |
|    | Basis Weight (g/m <sup>2</sup> ) | 45.0                              | 45.1   | 45.8   |
|    | Caliper (mm)                     | 0.46                              | 0.42   | 0.46   |
|    | Bulk (cm <sup>3</sup> /g)        | 10.3                              | 9.09   | 10.0   |
| 35 | Max. Cup Crush Load (N)          | 0.876                             | 1.14   | 1.09   |
|    | Cup Crush Energy (J)             | 0.0141                            | 0.0176 | 0.0161 |
|    | Dry Burst (N)                    | 2.30                              | 2.61   | 2.06   |
|    | MD Dry Tensile Strength (N/m)    | 194                               | 265    | 221    |
|    | CD Dry Tensile Strength (N/m)    | 127                               | 183    | 134    |
| 40 | MD:CD Tensile Ratio              | 1.53                              | 1.45   | 1.65   |
|    | MD Stretch                       | 14.6                              | 15.0   | 15.0   |
|    | CD Stretch                       | 4.6                               | 4.1    | 4.7    |
|    | MD TEA (J/m <sup>2</sup> )       | 11.5                              | 15.9   | 13.1   |
|    | CD TEA (J/m <sup>2</sup> )       | 3.5                               | 4.1    | 3.6    |

TABLE 2

|  |                                  | Properties of Single-Layer Tissues |        |        |       |       |        |
|--|----------------------------------|------------------------------------|--------|--------|-------|-------|--------|
|  |                                  | Tissue Sample                      |        |        |       |       |        |
|  |                                  | 4                                  | 5      | 6      | 7     | 8     | 9      |
|  | First Fibers (% tissue fibers)   | 70                                 | 70     | 70     | 80    | 70    | 70     |
|  | Second Fibers (% tissue fibers)  | 30                                 | 30     | 30     | 20    | 30    | 30     |
|  | SEPF (% of second fibers)        | 0                                  | 10     | 10     | 10    | 10    | 0      |
|  | Refining Energy (kWh/t)          | 80.3                               | 79.3   | 41.4   | 82    | 80.7  | 121    |
|  | TAD Roll 1 Propane Flow (kg/hr)  | 115                                | 111    | 113    | 112   | 107   | 113    |
|  | TAD Roll 2 Propane Flow (kg/hr)  | 70.6                               | 72.2   | 71     | 69.8  | 68.2  | 70.8   |
|  | Total TAD Propane Flow (kg/hr)   | 185.6                              | 183.2  | 184    | 181.8 | 175.2 | 183.8  |
|  | Yankee Dryer Steam Flow (kg/hr)  | 1038                               | 1067   | 1033   | 1013  | 937   | 1039   |
|  | Basis Weight (g/m <sup>2</sup> ) | 44.7                               | 45.9   | 45.1   | 45.2  | 41.0  | 46.7   |
|  | Caliper (mm)                     | 0.43                               | 0.42   | 0.42   | 0.44  | 0.41  | 0.41   |
|  | Bulk (cm <sup>3</sup> /g)        | 10.0                               | 9.09   | 9.09   | 10.0  | 10.0  | 0.11   |
|  | Max. Cup Crush Load (N)          | 1.030                              | 1.27   | 1.09   | 1.06  | 1.03  | 1.39   |
|  | Cup Crush Energy (J)             | 0.0161                             | 0.0185 | 0.0171 | 0.016 | 0.016 | 0.0214 |
|  | Dry Burst (N)                    | 2.11                               | 2.62   | 2.05   | 1.54  | 2.47  | 2.83   |

TABLE 2-continued

|                               | Properties of Single-Layer Tissues |      |       |      |      |      |
|-------------------------------|------------------------------------|------|-------|------|------|------|
|                               | Tissue Sample                      |      |       |      |      |      |
|                               | 4                                  | 5    | 6     | 7    | 8    | 9    |
| MD Dry Tensile Strength (N/m) | 211                                | 300  | 243   | 178  | 233  | 303  |
| CD Dry Tensile Strength (N/m) | 120                                | 170  | 138   | 113  | 132  | 168  |
| MD:CD Tensile Ratio           | 1.76                               | 1.76 | 1.76  | 1.58 | 1.77 | 1.8  |
| MD Stretch                    | 13.8                               | 14.7 | 14.40 | 14.3 | 14   | 14.3 |
| CD Stretch                    | 4.8                                | 4.7  | 4.8   | 4.4  | 4.6  | 4.6  |
| MD TEA (J/m <sup>2</sup> )    | 12.3                               | 18.2 | 14.3  | 10.9 | 13.3 | 17.4 |
| CD TEA (J/m <sup>2</sup> )    | 3.3                                | 4.5  | 3.8   | 3.0  | 3.4  | 4.3  |

The tissue samples that included SEPF were, in general, stronger than the controls. For example, Tissue Samples 2 and 5—which except for the inclusion of SEPF were the same as Tissue Samples 1 and 4, respectively—had a tensile strength that was 37%-44% and 42% stronger, respectively, than the corresponding control. However, Tissue Samples 2 and 5 were not as soft as their corresponding controls, as evidenced by their higher maximum cup crush loads and cup crush energies. The second fibers in Tissue Samples 3 and 6 were refined using less refining energy than those used in Tissue Samples 1 and 4, respectively. Despite the lower refining energy, Tissue Samples 3 and 6 were stronger than their corresponding controls; however, Tissue Sample 3 did not have a softness comparable to that of Tissue Sample 1.

Tissue Sample 7—which had a larger proportion of first fibers than the other samples—and Tissue Sample 8—which had a lower basis weight than the other samples—had a comparable softness to the control (Tissue Sample 4). Tissue Sample 8 had a higher dry tensile strength than the control; Tissue Sample 7 did not.

To make Tissue Sample 2, less propane was used to heat the air for the TAD rolls but more steam was used to heat the Yankee dryer, compared to Tissue Sample 1. For the single-layer tissues, as compared to the control, less propane was used when making each of the tissues that included SEPF and, of those, less steam was used for Tissue Samples 6-8. Tissue Sample 8 had the lowest total propane and steam flows of the single-layer tissues. That some of the SEPF tissue samples were easier to dry than the controls was unexpected, given the high WRV of SEPF.

### Example 2

Fifteen two-ply paper towel samples were made using a TAD process: two controls comprising no SEPF (Towel Samples 1 and 2), seven samples in which 5% of the second fibers were SEPF (Towel Samples 3-9), and six samples in which 10% of the second fibers were SEPF (Samples 10-15). Each of the samples comprised first fibers that were BEK fibers, second fibers that included NBSK fibers and soft-wood SEPF (except for Towel Sample 1, which had no SEPF), and third fibers that were SBSK fibers, where 25% of the fibers of the paper towel, by weight, were the third fibers. To form each of the samples, a furnish comprising the second fibers was beaten with a mechanical refiner before being combined with a furnish comprising the first and third fibers. Two wet strength resins—PAE and carboxymethyl cellulose—were added to the furnishes. For each of the plies, the combined furnishes were used to form a single-layer web that was dewatered to make the ply. As with Example 1, dewatering was achieved by vacuums and through-air drying. The TAD system included two TAD rolls

15 and a Yankee dryer—air for each of the TAD rolls was heated by burning propane and the Yankee dryer was heated with steam. The two plies were laminated and embossed to form the towel.

20 The proportions of first and second fibers, refining energy, amount of wet strength resins, and basis weight were varied. Towel properties—including caliper, bulk, air permeability, burst, wet burst, water drop absorbency, and machine direction and cross-direction stiffness, tensile strength, wet tensile strength, stretch, and TEA—were measured. TABLE 3 sets forth the results for Towel Samples 1 and 2, TABLE 4 sets forth the results for Towel Samples 3-9, and TABLE 5 sets forth the results for Towel Samples 10-15.

TABLE 3

|                                                        | Properties of Control Towels |                |
|--------------------------------------------------------|------------------------------|----------------|
|                                                        | Towel Sample 1               | Towel Sample 2 |
| 35                                                     |                              |                |
| BEK (% towel fibers)                                   | 20                           | 20             |
| NBSK (% towel fibers)                                  | 55                           | 55             |
| 40 SBSK (% towel fibers)                               | 25                           | 25             |
| Refining Energy (kWh/t)                                | 50.4                         | 80.8           |
| Basis Weight (g/m <sup>2</sup> )                       | 56.5                         | 57.1           |
| TAD Roll 1 Propane Flow (kg/hr)                        | 151                          | 148            |
| TAD Roll 2 Propane Flow (kg/hr)                        | 79                           | 75.6           |
| 45                                                     |                              |                |
| Total TAD Propane Flow (kg/hr)                         | 230                          | 223.6          |
| Yankee Dryer Steam Flow (kg/hr)                        | 1028                         | 1035           |
| PAE (kg/t)                                             | 10                           | 10             |
| Carboxymethyl Cellulose (kg/t)                         | 2                            | 2              |
| 50 Caliper (mm)                                        | 0.88                         | 0.88           |
| Bulk (cm <sup>3</sup> /g)                              | 15.6                         | 15.4           |
| Air Permeability (cm <sup>3</sup> /s·cm <sup>2</sup> ) | 33.6                         | 30.8           |
| MD Stiffness (mN)                                      | 2012                         | 2264           |
| CD Stiffness (mN)                                      | 1430                         | 1797           |
| Handle (mN)                                            | 6883                         | 8121           |
| 55 Dry Burst (N)                                       | 10.4                         | 11.7           |
| Wet Burst (N)                                          | 3670                         | 3994           |
| Water Drop Absorbency (s)                              | 4.7                          | 5.0            |
| MD Dry Tensile Strength (N/m)                          | 571                          | 659            |
| CD Dry Tensile Strength (N/m)                          | 399                          | 444            |
| 60 MD Wet Tensile Strength (N/m)                       | 183                          | 206            |
| CD Wet Tensile Strength (N/m)                          | 123                          | 133            |
| MD Stretch                                             | 17.2                         | 17.1           |
| CD Stretch                                             | 9.5                          | 9.6            |
| MD TEA (J/m <sup>2</sup> )                             | 42.8                         | 49.7           |
| 65 CD TEA (J/m <sup>2</sup> )                          | 19.6                         | 21.7           |

TABLE 4

| Properties of Towels in Which 5% of the Second Fibers were SEPF |              |       |       |       |       |       |       |
|-----------------------------------------------------------------|--------------|-------|-------|-------|-------|-------|-------|
|                                                                 | Towel Sample |       |       |       |       |       |       |
|                                                                 | 3            | 4     | 5     | 6     | 7     | 8     | 9     |
| BEK (% towel fibers)                                            | 20           | 20    | 35    | 20    | 20    | 20    | 20    |
| Second Fibers (% towel fibers)                                  | 55           | 55    | 40    | 55    | 55    | 55    | 55    |
| SBSK (% towel fibers)                                           | 25           | 25    | 25    | 25    | 25    | 25    | 25    |
| Refining Energy (kWh/t)                                         | 49.9         | 25.2  | 50.8  | 50.2  | 49.9  | 49.0  | 0     |
| TAD Roll 1 Propane Flow (kg/hr)                                 | 147          | 147   | 147   | 145   | 150   | 150   | 146   |
| TAD Roll 2 Propane Flow (kg/hr)                                 | 74.2         | 73.4  | 76.7  | 75.2  | 74.6  | 71.2  | 69.7  |
| Total TAD Propane Flow (kg/hr)                                  | 221.2        | 220.4 | 223.7 | 220.2 | 224.6 | 221.2 | 215.7 |
| Yankee Dryer Steam Flow (kg/hr)                                 | 1021         | 995   | 1006  | 1007  | 1006  | 990   | 962   |
| Basis Weight (g/m <sup>2</sup> )                                | 55.6         | 54.7  | 55.3  | 51.6  | 54.2  | 53.3  | 54.3  |
| PAE (kg/t)                                                      | 10           | 10    | 10    | 10    | 6     | 14    | 14    |
| Carboxymethyl Cellulose (kg/t)                                  | 2            | 2     | 2     | 2     | 1.2   | 2.8   | 2.8   |
| Caliper (mm)                                                    | 0.91         | 0.91  | 0.90  | 0.89  | 0.87  | 0.90  | 0.89  |
| Bulk (cm <sup>3</sup> /g)                                       | 16.4         | 16.7  | 16.40 | 17.2  | 16.1  | 16.9  | 16.4  |
| Air Permeability (cm <sup>3</sup> /s-cm <sup>2</sup> )          | 32.6         | 34.9  | 31.8  | 40.1  | 34.5  | 36.6  | 38.6  |
| MD Stiffness (mN)                                               | 2147         | 1885  | 1934  | 1857  | 1880  | 2256  | 2006  |
| CD Stiffness (mN)                                               | 1673         | 1456  | 1456  | 1257  | 1284  | 1499  | 1319  |
| Handle (mN)                                                     | 7639         | 6682  | 6780  | 6229  | 6329  | 7511  | 6651  |
| Dry Burst (N)                                                   | 10.8         | 9.78  | 8.71  | 9.63  | 9.08  | 10.5  | 8.19  |
| Wet Burst (N)                                                   | 4276         | 3396  | 3186  | 3168  | 2951  | 4029  | 3146  |
| Water Drop Absorbency (s)                                       | 5.2          | 5.2   | 4.7   | 5.0   | 5.3   | 5.0   | 5.2   |
| MD Dry Tensile Strength (N/m)                                   | 610          | 506   | 492   | 517   | 526   | 581   | 429   |
| CD Dry Tensile Strength (N/m)                                   | 423          | 358   | 352   | 349   | 342   | 395   | 300   |
| MD Wet Tensile Strength (N/m)                                   | 204          | 167   | 166   | 164   | 154   | 195   | 152   |
| CD Wet Tensile Strength (N/m)                                   | 136          | 119   | 107   | 106   | 98    | 128   | 101   |
| MD Stretch                                                      | 16.4         | 16.1  | 16.1  | 17.4  | 17.6  | 17.4  | 17.0  |
| CD Stretch                                                      | 3.6          | 9.5   | 9.4   | 9.7   | 9.3   | 10.0  | 9.9   |
| MD TEA (J/m <sup>2</sup> )                                      | 43.8         | 35.5  | 35.2  | 38.7  | 40.5  | 43.9  | 31.6  |
| CD TEA (J/m <sup>2</sup> )                                      | 20.2         | 17.4  | 16.7  | 17.1  | 16.6  | 19.9  | 15.2  |

TABLE 5

| Properties of Towels in Which 10% of the Second Fibers were SEPF |              |       |       |      |       |       |
|------------------------------------------------------------------|--------------|-------|-------|------|-------|-------|
|                                                                  | Towel Sample |       |       |      |       |       |
|                                                                  | 10           | 11    | 12    | 13   | 14    | 15    |
| BEK (% towel fibers)                                             | 20           | 20    | 20    | 20   | 45    | 20    |
| Second Fibers (% towel fibers)                                   | 55           | 55    | 55    | 55   | 30    | 55    |
| SBSK (% towel fibers)                                            | 25           | 25    | 25    | 25   | 25    | 25    |
| Refining Energy (kWh/t)                                          | 48.7         | 49.0  | 50.2  | 50.5 | 50.4  | 50.0  |
| TAD Roll 1 Propane Flow (kg/hr)                                  | 147          | 151   | 147   | 143  | 147   | 143   |
| TAD Roll 2 Propane Flow (kg/hr)                                  | 74.7         | 77.8  | 77.7  | 70   | 73.5  | 71.6  |
| Total TAD Propane Flow (kg/hr)                                   | 221.7        | 228.8 | 224.7 | 213  | 220.5 | 214.6 |
| Yankee Dryer Steam Flow (kg/hr)                                  | 1030         | 1031  | 1030  | 981  | 1002  | 984   |
| Basis Weight (g/m <sup>2</sup> )                                 | 55.1         | 55.2  | 55.8  | 51.0 | 55.3  | 50.3  |
| PAE (kg/t)                                                       | 10           | 10    | 14    | 14   | 14    | 10    |
| Carboxymethyl Cellulose (kg/t)                                   | 2            | 2     | 2.8   | 2.8  | 2.8   | 2     |
| Caliper (mm)                                                     | 0.88         | 0.90  | 0.90  | 0.89 | 0.91  | 0.85  |
| Bulk (cm <sup>3</sup> /g)                                        | 15.9         | 16.4  | 16.1  | 17.2 | 16.4  | 16.9  |
| Air Permeability (cm <sup>3</sup> /s-cm <sup>2</sup> )           | 31.4         | 30.6  | 30.3  | 40.3 | 30.9  | 41.1  |
| MD Stiffness (mN)                                                | 2044         | 2435  | 2628  | 2359 | 2363  | 2279  |
| CD Stiffness (mN)                                                | 1503         | 1809  | 1766  | 1522 | 1548  | 1633  |
| Handle (mN)                                                      | 7094         | 8489  | 8787  | 7763 | 7809  | 7825  |
| Dry Burst (N)                                                    | 10.1         | 10.5  | 11.3  | 9.83 | 8.28  | 9.76  |
| Wet Burst (N)                                                    | 3958         | 3780  | 4692  | 4342 | 2860  | 3596  |
| Water Drop Absorbency (s)                                        | 5.0          | 5.20  | 5.2   | 5.3  | 5.2   | 5.2   |
| MD Dry Tensile Strength (N/m)                                    | 582          | 574   | 637   | 546  | 435   | 524   |
| CD Dry Tensile Strength (N/m)                                    | 399          | 415   | 442   | 392  | 322   | 362   |
| MD Wet Tensile Strength (N/m)                                    | 192          | 211   | 237   | 211  | 160   | 173   |
| CD Wet Tensile Strength (N/m)                                    | 130          | 135   | 147   | 137  | 109   | 116   |
| MD Stretch                                                       | 17.5         | 17.4  | 17.7  | 17.4 | 16.8  | 17.3  |
| CD Stretch                                                       | 9.6          | 9.6   | 9.7   | 10.0 | 9     | 9.9   |
| MD TEA (J/m <sup>2</sup> )                                       | 44.4         | 43.1  | 49.1  | 41.0 | 32.8  | 39.1  |
| CD TEA (J/m <sup>2</sup> )                                       | 19.4         | 20.0  | 21.5  | 19.7 | 14.5  | 18.1  |

During production, the second fibers were refined using more energy for the second control (Towel Sample 2) than for the first control (Towel Sample 1). A similar level of refining was used for all SEPF-containing samples (except for Towel Samples 4 and 9) as was used for Towel Sample 1.

As with the tissues, the towel samples that included SEPF were, in general, stronger than the controls, all else being equal. For example, Towel Samples 3 and 10—which except for the inclusion of SEPF were the same as Towel Sample 1—had wet bursts that were 7% and 8% larger, respectively, than the wet burst of Towel Sample 1. However, these towels were not as soft as Towel Sample 1, as reflected by the larger handles thereof.

Compared to Towel Samples 1, less refining energy was used to refine the second fibers of Towel Sample 4, Towel Sample 5 had a lower proportion of second fibers, Towel Sample 6 had a lower basis weight, and Towel Sample 7 used less wet strength resin. These towel samples were not as strong as Towel Sample 1, as reflected by their lower wet bursts, and only some (e.g., Towel Samples 6 and 7) exhibited improved softness (e.g., lower handle). For example, Towel Sample 5—which incorporated fewer second fibers—exhibited little, if any, improvement in softness.

More wet strength resin was used in Towel Samples 8, 9, 25 and 12-14, compared to Towel Samples 1 and 2. Additionally, compared to Towel Samples 1 and 2, the second fibers of Towel Sample 9 were not refined, Towel Sample 13 had a lower basis weight, and Towel Sample 14 had a lower proportion of second fibers. Increasing the amount of wet 30 strength resin tended to increase strength at the expense of softness, as reflected by the higher wet bursts and handles of Towel Samples 8 and 12. Compared to Towel Sample 1, Towel Sample 9 was softer but also had lower strength, and Towel Sample 14 was both weaker and less soft. Towel 35 Sample 13 had a higher wet burst than the Towel Sample 1, and while it was less soft (e.g., had a higher handle) than Towel Sample 1, it was softer (e.g., had a lower handle) than Towel Sample 12.

For all samples that incorporated SEPF, the total propane 40 used to heat the air for the TAD rolls was lower than that used when making Towel Sample 1. And, compared to Towel Sample 1, for all SEPF-containing samples except for Towel Samples 10 and 12 less steam was used to heat the Yankee dryer. This again was an unexpected result because the SEPF—due to its high WRV—was anticipated to make 45 drying harder, rather than easier, compared to the control.

The above specification and examples provide a complete 50 description of the structure and use of illustrative embodiments. Although certain embodiments have been described above with a certain degree of particularity, or with reference to one or more individual embodiments, those skilled in the art could make numerous alterations to the disclosed 55 embodiments without departing from the scope of this invention. As such, the various illustrative embodiments of the products, systems, and methods are not intended to be limited to the particular forms disclosed. Rather, they include all modifications and alternatives falling within the scope of the claims, and embodiments other than the one shown may include some or all of the features of the 60 depicted embodiment. For example, elements may be omitted or combined as a unitary structure, and/or connections may be substituted. Further, where appropriate, aspects of any of the examples described above may be combined with aspects of any of the other examples described to form 65 further examples having comparable or different properties and/or functions, and addressing the same or different prob-

lems. Similarly, it will be understood that the benefits and advantages described above may relate to one embodiment or may relate to several embodiments.

The claims are not intended to include, and should not be interpreted to include, means-plus- or step-plus-function limitations, unless such a limitation is explicitly recited in a given claim using the phrase(s) "means for" or "step for," respectively.

The invention claimed is:

1. A tissue comprising:

a first plurality of first fibers that are hardwood fibers; a second plurality of second fibers including softwood fibers and surface enhanced pulp fibers (SEPF) having a length weighted average fiber length that is at least 0.20 millimeters (mm), wherein the SEPF are made by refining a pulp feed, the refining including for each of one or more mechanical refiners:

introducing the pulp feed between two refining elements of the refiner, each of the refining elements comprising:

a plurality of bars, each protruding from a surface of the refining element and having a width that is less than or equal to 1.3 mm; and

a plurality of grooves defined by the bars, each having a width that is less than or equal to 2.5 mm; and

rotating at least one of the refining elements; wherein refining the pulp feed is performed such that the refiner(s) consume at least 300 kilowatt-hours (kWh) per ton of fiber in the pulp feed; and

two or more fiber layers that include:

one or more first fiber layers that comprise the first fibers, at least one of the first fiber layer(s) defining one of opposing upper and lower surfaces of the tissue; and

one or more second fiber layers that comprise the second fibers;

wherein by weight:

at least 90% of the second fibers are the softwood fibers; and

between 1% and 10% of the second fibers are the SEPF.

2. The tissue of claim 1, wherein by weight: between 50% and 80% of the fibers of the tissue are the first fibers; and

at least 20% of the fibers of the tissue are the second fibers.

3. The tissue of claim 1, wherein:

the one or more first fiber layers comprise two first fiber layers, each defining a respective one of the upper and lower surfaces of the tissue; and

each of the one or more second fiber layers is disposed between the two first fiber layers.

4. The tissue of claim 1, wherein a total basis weight of the second fiber layer(s) is between 25% and 35% of the total basis weight of the first fiber layer(s).

5. The tissue of claim 1, wherein by weight:

at least 90% of the fibers of the first fiber layer(s) are the first fibers; and

at least 90% of the fibers of the second fiber layer(s) are the second fibers.

6. The tissue of claim 1, wherein:

a maximum cup crush load of the tissue is less than or equal to 1.0 Newton (N); and

a tensile strength of the tissue is greater than or equal to 200 N/m.

**21**

7. The tissue of claim 1, wherein:  
the tissue comprises one or more plies; and  
the basis weight of the tissue is less than or equal to 21  
grams per square meter (gsm) per ply.
8. The tissue of claim 1, wherein the SEPF are softwood  
fibers.
9. The tissue of claim 1, wherein by weight:  
between 65% and 75% of the fibers of the tissue are the  
first fibers; and  
at least 25% of the fibers of the tissue are the second  
fibers.
10. The tissue of claim 1, wherein the length weighted  
average fiber length of the SEPF is at least 0.20 mm and the  
average hydrodynamic specific surface area of the SEPF is  
at least 10 m<sup>2</sup>/g.
11. The tissue of claim 1, wherein the hardwood fibers of  
the first fibers comprise bleached eucalyptus fibers.
12. The tissue of claim 1, wherein the softwood fibers of  
the second fibers comprise northern bleached softwood kraft  
fibers.
13. A tissue comprising:  
a first plurality of first fibers that are hardwood fibers;  
a second plurality of second fibers including softwood  
fibers and surface enhanced pulp fibers (SEPF) having  
a length weighted average fiber length that is at least  
0.20 millimeters (mm), wherein the SEPF are made by  
refining a pulp feed, the refining including for each of  
one or more mechanical refiners:  
introducing the pulp feed between two refining ele-  
ments of the refiner, each of the refining elements  
comprising:  
a plurality of bars, each protruding from a surface of  
the refining element and having a width that is less  
than or equal to 1.3 mm; and  
a plurality of grooves defined by the bars, each  
having a width that is less than or equal to 2.5 mm;  
and  
rotating at least one of the refining elements;  
wherein refining the pulp feed is performed such that  
the refiner(s) consume at least 300 kilowatt-hours  
(kWh) per ton of fiber in the pulp feed; and  
two or more plies;  
wherein:  
by weight:  
between 50% and 80% of the fibers of the tissue are  
the first fibers and at least 20% of the fibers of the  
tissue are the second fibers;

**22**

- at least 90% of the second fibers in a first ply of the  
two or more plies are the softwood fibers; and  
between 1% and 10% of the second fibers in the first  
ply are the SEPF; and  
the basis weight of the tissue is less than or equal to 21  
grams per square meter (gsm) per ply.
14. The tissue of claim 13, wherein:  
a maximum cup crush load of the tissue is less than or  
equal to 1.06 Newtons (N); and  
a tensile strength of the tissue is greater than or equal to  
220 N/m.
15. A method of making a tissue, the method comprising:  
refining a pulp feed to generate surface enhanced pulp  
fibers (SEPF) by:  
for each of one or more mechanical refiners:  
introducing the pulp feed between two refining ele-  
ments of the mechanical refiner, each refining  
element comprising:  
a plurality of bars, each bar protruding from a  
surface of the refining element and having a  
width that is less than or equal to 1.3 mm; and  
a plurality of grooves defined by the bars, each  
groove having a width that is less than or equal  
to 2.5 mm; and  
rotating at least one of the refining elements,  
wherein refining the pulp feed is performed such that  
the one or more mechanical refiners consume at least  
300 kilowatt-hours (kWh) per ton of fiber in the pulp  
feed;  
providing a first plurality of first fibers that are hardwood  
fibers;  
generating a second plurality of second fibers by mixing  
together softwood fibers and the SEPF;  
forming one or more first fiber layers comprising the first  
fibers, at least one of the one or more first fiber layers  
defining one of opposing upper and lower surfaces of  
the tissue;  
forming one or more second fiber layers comprising the  
second fibers; and  
disposing each of the one or more second fiber layers  
between the one or more first fiber layers,  
wherein by weight:  
at least 90% of the second fibers are the softwood  
fibers, and  
between 1% and 10% of the second fibers are the  
SEPF.

\* \* \* \* \*